

May 2, 1933.

E. S. SMITH

1,907,094

PROCESS FOR PRODUCING CLOUD EFFECTS IN ENAMELS

Filed Nov. 23, 1932



Fig. I



Fig. II

Earle S. Smith  
INVENTOR

BY *O. Marshall*  
ATTORNEY

## UNITED STATES PATENT OFFICE

EARLE S. SMITH, OF TOLEDO, OHIO, ASSIGNOR TO THE TOLEDO PORCELAIN ENAMEL PRODUCTS COMPANY, OF TOLEDO, OHIO, A CORPORATION OF OHIO

## PROCESS FOR PRODUCING CLOUD EFFECTS IN ENAMELS

Application filed November 23, 1932. Serial No. 643,970.

This invention relates to processes for producing cloud effects in enamels and particularly to a process for producing effects having the appearance of clouds formed in light 5 wisps through which a sky-like background is visible, thus simulating the effect of a cirrus clouded sky.

Another object is the provision of a process for producing light cloud effects in which 10 cloud wisps are given a slightly fibrous "mackerel sky" effect.

Other objects and advantages will be apparent from the following description, in which reference is had to the accompanying 15 drawing in which Figure I illustrates the appearance of a panel upon which my enameling process has been partially carried out and Figure II illustrates the panel after a succeeding step of the process has been applied 20 thereto. Owing to the impracticability of reproducing the beauty of the final effect, no attempt has been made to illustrate the panel after the final step.

In carrying out the process of my invention, a metal, preferably iron or steel, article 25 or piece to be enameled, after proper cleaning is dipped, sprayed or otherwise covered with a first or so-called "ground" coat of vitreous enamel frit the color of which is not important 30 so far as ultimate appearance is concerned. If the ground coat is applied by a wet process it is then thoroughly dried. The ground coat of vitreous enamel is next fused to the metal in an enameling furnace.

35 When the article has cooled it is sprayed or dipped to coat it solidly with enamel frit to form a background of proper color, such, for example, as sky blue.

While the coat of solid color is still wet it is 40 speckled, by means of a splatter gun or otherwise, with numerous small spots of enamel of another color, giving it an appearance resembling that of the panel illustrated in Figure I of the drawing. The spots, however, 45 instead of being black on a white background, may be white on a blue background, or any other combination of colors may be selected.

While the spattered surface is still wet it is 50 brushed in one direction with a wire or stiff bristle brush or comb, the wires, bristles or

teeth of which are spaced apart so that the surface of the wet enamel is furrowed and the colors are streaked into each other; the surface thus taking on the appearance illustrated in Figure II of the drawing. 55

While the outer coating is still wet and somewhat fluid the article is jarred or jolted. This results in smoothing out the furrows left by the brushing or combing operation and giving the streaked color a light, fluffy, 60 delicate appearance, with the fibrous structure and feather-like form of a cirrus clouded sky.

The coating is then thoroughly dried and finally fused to the ground coat, the fusing 65 operation further enhancing the beauty of the clouded coating.

Although I have illustrated the steps of my process in black and white and have described the process as utilizing blue and white, 70 the effect may be obtained with any selected colors. The embodiment of my invention herein described is to be regarded as illustrative only, and it is to be understood that the invention is susceptible to variation, modification and change within the spirit and 75 scope of the subjoined claims.

Having described my invention, I claim:

1. In an enameling process, the steps of applying to a surface a solid wet coat of vitreous enamel frit of one color, speckling said coat with wet vitreous enamel frit of another color, streaking said coat by a brushing operation, jarring said coat to produce a cirrus clouded effect, drying, and fusing said coat 85 to said surface.

2. In an enameling process, the steps of applying to a surface a ground coat, fusing said ground coat thereto, applying to said ground coat a solid wet coat of vitreous enamel frit 90 of one color, speckling said coat with wet vitreous enamel frit of another color, streaking said coat by a brushing operation, jarring said coat to produce a cirrus clouded effect, drying, and fusing said coat to said surface. 95

EARLE S. SMITH.